

# UNITED STATES PATENT OFFICE.

FOSTER MILLIKEN, OF LAWRENCE, NEW YORK, ASSIGNOR TO FOSTER MILLIKEN,  
S. FULLERTON WEAVER, AND JAMES M. REPLIER, TRUSTEES.

## ALLOY.

1,351,673.

Specification of Letters Patent. Patented Aug. 31, 1920.

No Drawing.

Application filed October 8, 1919. Serial No. 329,375.

*To all whom it may concern:*

Be it known that I, FOSTER MILLIKEN, a citizen of the United States, and a resident of Lawrence, in the county of Nassau and State of New York, have invented a new and Improved Alloy, of which the following is a full, clear, and exact description.

The object of the invention is to provide a new and improved alloy more especially designed for use in mine water valves and other devices subjected to weak acids.

The alloy consists of the following metals, in approximately the proportions specified, namely:

15 Copper ----- 42 to 52 per cent.  
Nickel ----- 22 to 28 " "  
Lead ----- 22 to 30 " "

These metals are melted together and cast in the usual way, and the resultant alloy is especially serviceable to resist the corrosive action of weak acids, such, for instance, as mine water containing 4 to 600 grains of sulfuric acid per gallon, or tartaric acid under 10%, or phosphoric acid under 10%.

I claim:

1. An alloy formed from copper 42 to 52 per cent., nickel 22 to 28 per cent., and lead 22 to 30 per cent.

2. An alloy containing copper, nickel, and lead, of which the percentage of the nickel and the lead is approximately equal and approximately one-half of that of the copper.

FOSTER MILLIKEN.